

Patented Feb. 1, 1927.

1,616,062

# UNITED STATES PATENT OFFICE.

EMIL E. NOVOTNY AND CHARLES J. ROMIEUX, OF PHILADELPHIA, PENNSYLVANIA,  
ASSIGNORS TO JOHN STOGDELL STOKES, OF SPRING VALLEY FARMS, HUNTING-  
DON VALLEY POST OFFICE, PENNSYLVANIA.

## METHOD OF WATERPROOFING VULCANIZED FIBER.

No Drawing.

Application filed September 4, 1923. Serial No. 660,952.

This invention relates to a method of waterproofing vulcanized fiber, viscose and similar materials of cellulose origin which are thereby formed into sheets or plastic materials.

More particularly stated, this invention comprises a method of treating fibrous materials which have been previously impregnated with, or have had incorporated therein, a synthetic resinous product such as, for example, the phenolic condensation product made of phenol and furfural and known generally in the trade as durite. This material has very high mechanical and dielectric strength and is described in patent issued to Novotny and Kendall, Number 1,398,146, issued November 22, 1921, and the co-pending application of Novotny and Kendall, Serial Number 501,273, filed September 17, 1921. In this patent and the application referred to there have been shown several useful forms of phenolic condensation products which are particularly well suited for this purpose.

The step of impregnating or incorporating in the fibrous structure a suitable cementitious binder which is not subsequently altered or dissolved out of the structure by the converting agent acting upon the cellular material, permits of an intimate combination of binder with the eventually altered cellular structure after it has been treated as in the well-known art of paper vulcanization. It is already well-known in the art that cellular structures may be altered by various means as in the production of vulcanized fiber or viscose. For example, when vulcanized fiber is produced the cellulose tissue is gelatinized or subjected to hydrolysis in the presence of a material such as zinc chloride. Other steps, of course, can be utilized, such as, for example, a treatment with cold sulphuric acid or cupro-ammonium solution. As the art of altering cellulose bodies into jellylike or gelatinous substances is well-known, it does not require further mention here.

We are aware, also, that it has been proposed to impregnate vulcanized fiber with a phenolic condensation product after such vulcanized fiber had been formed. This, however, is not the nature of our improvement. It has been found practically impossible to thoroughly and properly impreg-

nate a sheet of vulcanized fiber inasmuch as the material is non-porous or has more of the characteristics of a gel and therefore the resin cannot be absorbed by the material.

We find, however, that where a sheet of paper is impregnated with a varnish or resinous body and is not pressed or compacted to a greater extent than necessary to remove surplus material, the paper or sheetlike structure will be capable of absorbing large quantities of water, and this to a much greater extent than if the fiber or cellular structure were gelatinized or altered as by hydrolysis in the vulcanized fiber process. This facility of the resin impregnated or incorporated sheet of taking up various quantities of water makes it possible to introduce therein the modifying medium such as zinc chloride which causes the hydrolysis of the sheet, and which therefore, after the zinc chloride is removed, results in an intimate mixture of gelatinized or altered or hydrolyzed cellulose and binder, reinforcing medium, or water-proofing agent therefor.

Likewise, this method permits of the treatment of thicker sheets of paper than would be possible if the waterproofing material or binder were to be introduced subsequently by impregnation into the previously hydrolyzed cellulose. Likewise, thick sheets of laminated fiber can be produced rapidly with only a short washing operation inasmuch as such sheets can be treated practically on a continuous process machine, and after being dried they may be cemented together by the coating of the binder on the surface or the cementing action of the incorporated binder coming to the surface upon being formed as by the combined action of heat and pressure.

To make our method clear it may be stated that the fiber such as paper, cloth or other cellulose material is impregnated with the durite, dissolved in a suitable solvent such as, for example, alcohol, this solution being of proper strength to give the percentage of impregnation desired. The sheet may be dried but preferably this operation is dispensed with. The web is submerged in a water bath which removes therefrom the excess alcohol and causes the fibrous body to be thoroughly wetted with water. The web is now run into another vat containing

the zinc chloride solution which penetrates into the fibrous structure very readily because of the affinity it has for the water present in the fiber, and the fiber is thereby 5 quickly hydrolyzed. The web is subsequently washed to remove the zinc chloride or other altering media, is dried at low temperature, and may be rolled to be subsequently cut into sheets or used in any desired manner.

As another example of incorporating the binder or resinous body with the fibrous cellulose material, we can proceed as follows:

To the paper pulp in the beaters is added 15 a suitable percentage of resinous material which may be caused to be dissolved in the alkaline water present in the beaters, or such resinous material may be added to the pulp after having been previously dissolved in a 20 suitable solvent. After a beating of say from five minutes to one hour, or as may be deemed desirable for the particular end product to be obtained, we add a suitable precipitant, for example, ammonium sulphate. Since the precipitate thus formed is 25 very bulky, it is widely dispersed and readily clings to the fiber. The beaten mass of fibers is now in suitable condition to be transferred to the sheet forming device or 30 paper making machine where it is formed into sheetlike products of various thicknesses in the usual and well-known manner. The sheets may be dried and rolled for subsequent hydrolyzing treatment or, if sufficiently strong in their wet condition, the 35 operation of forming the sheet and hydrolyzing may be a continuous process.

This laminated composite body may be rolled between heated rolls or pressed as between 40 the platens of a heated press to produce products of various degrees of hardness. When a binding material such as a potentially reactive resin, as, for example, durite, is used, the resin may be cured under 45 heat or under the combined action of heat and pressure so that it assumes its final infusible form. When this is done the product is of a hard, tough, and moisture-resistant nature. In this form it is well adapted for 50 being molded into various shapes and forms and may be used for the purpose of making bodies of sheetlike form for the mechanical and electrical arts.

Inasmuch as the fibrous structure has 55 been altered to a non-porous, non-fibrous body, and inasmuch as the binder is very thoroughly distributed throughout the structure, the products upon being formed, as under the action of heat and pressure, do 60 possess characteristics radically different from products where ordinary unaltered paper or cloth is impregnated with a resinous body such as durite or an endeavor is made to partially impregnate thin sheets 65 of vulcanized fiber with a varnishlike solu-

tion of such resin. As compared to the ordinary laminated phenolic condensation products, the material does not have the paper-like structure or basis but assumes rather a hornlike and tough structure. It is, 70 therefore, admirably suited in the mechanical arts where great toughness and strength are desired as an improvement on gear blanks, etc., made of ordinary vulcanized fiber or laminated phenolic products of 75 either paper or cloth. Furthermore, this material punches and shears cold more readily so that thicknesses of  $\frac{1}{8}$ " and over can be thus economically produced. The machining operations can likewise be more advantageously handled in a product where the fibrous structure has been altered as by vulcanization.

We do not limit ourselves specifically to a sheet like body inasmuch as it is readily understood that this product could be otherwise formed or comminuted into powdery form or that the fibrous or cellular material could be operated on in comminuted form and that the basis of impregnation before 90 the conversion of the product to its hydrolyzed form would hold true even in these powdery materials. We find that articles molded from this type of powdery material show greater toughness and permit machining operations to a much greater degree. The product is very compact and can therefore be easily handled in the molds and dies. It will readily be understood that in place of paper other structures formed of cellulose 100 can be employed, such as wood flour, corn cob cellulose, cloth and woven structures, etc.

Where we have herein described in the two examples methods of introducing durite, which is a condensation product of furfural, 105 we wish it to be understood that other synthetic resinous materials or phenolic condensation products may be used, such as those of formaldehyde, acetaldehyde, etc.

Further more, we do not limit ourselves 110 to the precise steps or method disclosed inasmuch as other equivalent methods could be used or some of the steps could be eliminated. For example, it is preferably, but not essential, to wet the sheet prior to introducing it into the vat containing the vulcanizing or altering medium; or, if preferred, the resinous body could be simply mixed in the beaters without going through the steps of dissolving the same in a suitable 120 solvent and then precipitating the resin out of solution. We have found that merely mixing the resinous material and preferably, but not necessarily, supplying a vehicle or suspending material, such as starch or gelatin, will answer the purpose for certain uses.

What we claim is—

1. The herein described method of waterproofing or reinforcing cellulose which comprises introducing a synthetic resin into 125

- the cellulose structure and subsequently treating such structure with a cellulose altering agent.
2. The herein described method of waterproofing or reinforcing cellulose which comprises introducing a phenolic condensation product into the cellulose structure and subsequently treating such structure with a cellulose altering agent.
3. The herein described method of waterproofing or reinforcing cellulose which comprises introducing a condensation product of phenol and furfural into the cellulose structure and subsequently treating such structure with a cellulose altering agent.
4. The herein described method of waterproofing or reinforcing cellulose which comprises introducing a resinoid phenolic condensation product into the cellulose structure, then treating such structure with a cellulose altering agent and then heating the same to convert the condensation product into its infusible state.
5. The herein described method of waterproofing or reinforcing cellulose which comprises impregnating or incorporating a resinoid phenolic condensation product into the cellulose structure, then treating such structure with a cellulose altering agent, and then heating and pressing the same to convert the condensation product and the cellulose body into a hard, strong and infusible structure.
6. The herein described method of waterproofing or reinforcing cellulose which comprises introducing a synthetic resinous body or waterproofing agent into the cellulose structure, subsequently treating such structure with a cellulose altering agent and applying heat and pressure to such structure to waterproof and reinforce the same.
7. The herein described method of waterproofing or reinforcing cellulose which comprises introducing a phenolic condensation product as a binder or waterproofing agent into the cellulose structure, subsequently treating such structure with a cellulose altering agent forming a body of laminated sheets so treated and heating and pressing the same to form a laminated body and thereby likewise waterproofing and reinforcing the same.

Signed at Philadelphia, in the county of Philadelphia, and State of Pennsylvania, this 1st day of September, A. D. 1923.

EMIL E. NOVOTNY.  
CHARLES J. ROMIEUX.